

# UNITED STATES PATENT OFFICE.

CLEMENT L. PERKINS, OF PITTSBURGH, PENNSYLVANIA, ASSIGNOR TO METALS RECOVERY COMPANY, OF NEW YORK, N. Y., A CORPORATION OF MAINE.

## FLOTATION OF MINERALS.

1,240,598.

Specification of Letters Patent. Patented Sept. 18, 1917.

No Drawing.

Application filed August 2, 1917. Serial No. 184,054.

To all whom it may concern:

Be it known that I, CLEMENT L. PERKINS, a citizen of the United States, residing at Pittsburgh, in the county of Allegheny, State of Pennsylvania, have invented certain new and useful Improvements in Flotation of Minerals, (Case B;) and I do hereby declare the following to be a full, clear, and exact description of the invention, such 10 as will enable others skilled in the art to which it appertains to make and use the same.

This invention relates to the concentration of minerals, such as sulfid ores and the like, (for example, chalcopyrite with a silicious gangue), by flotation, and is based upon the discovery that improved results can be obtained by carrying out the flotation operation with the addition to the ore or mineral pulp of xylidin (aminoxylen), either alone or with the addition of other agents promoting the flotation.

The xylidin may be used in the form of the commercial product which is made up of a mixture of the individual xylidins. Such commercial xylidin can be used in its crude or unrefined state.

In using the xylidin it may be added to the ore either alone or in admixture with other agents promoting the flotation, in any suitable manner, so that it will be thoroughly and uniformly distributed throughout the ore pulp. The mixture is then subjected to a flotation operation as in an ordinary Cal-low cell or in apparatus where the air is incorporated in the ore pulp by mechanical agitation. With some ore pulps it may be desirable to add either small amounts of acids or of alkalis, depending upon the nature of the ore pulp to be treated, but it will be evident that free acid should not be present to any appreciable extent when the xylidin is added. That is to say, if the ore pulp contains free acid, or if acid is preliminarily added thereto, the free acid should not be present when the xylidin is added, or should not be present to any appreciable extent such as would prejudice or destroy the effect of the xylidin, which is of a basic character, during the flotation operation.

With some ore pulps it is important not only to have no free acid present, but to

add sufficient free alkali to give a distinct alkaline reaction to the ore pulp during the 55 flotation operation. Small amounts of caustic alkali, such as sodium hydrate, or of alkali salts, such as sodium carbonate, may thus be added, in regulated amounts, to give the ore pulp the proper degree of alkalinity. 60

The amount of xylidin used may vary somewhat for example, between one-half pound or less and one and one-half pounds per ton of ore (that is, calculated on the weight of the ore and not of the ore pulp). 65 It is characteristic of the invention that the froth obtained is readily broken up and the xylidin recovered therefrom so that it is available for use in the treatment of further amounts of ore. That is to say, the circuit 70 water recovered from the concentrate and even that recovered from the tailings contains notable amounts of the xylidin which can thus be returned to the process with resulting economy in the amount required to 75 be added for subsequent operations.

The xylidin may be used alone to promote the flotation operation and high grades of concentrates obtained; and the resulting concentrates can be much more easily 80 separated by filtration than the common concentrates obtained by the use of oil as the flotation agent. The action of the xylidin may, however, be modified or supplemented by adding other agents (such as oils or non-oleaginous agents) which promote the flotation and which do not prejudicially affect the action of the xylidin. 85

In applying the xylidin, it may be introduced into the tube mill in which the ore is 90 being ground, or it may be otherwise introduced into the ore pulp in any suitable way, as, for instance, by dropping it into the ore pulp before it enters the flotation cell, or by first digesting it in hot water and mixing 95 the product with the ore pulp just before it enters the flotation cell.

What I claim is:

1. The method of effecting the concentration of minerals by flotation, which comprises adding to the mineral pulp a small amount of xylidin, and subjecting the resulting mixture to a flotation operation; substantially as described. 100
2. The method of effecting the concentration of minerals by flotation, which com- 105

prises adding to the mineral pulp a small amount of xylidin and other agents promoting the flotation, and subjecting the resulting mixture to a flotation operation; substantially as described.

3. The method of effecting the concentration of minerals by flotation, which comprises adding to the mineral pulp a small amount of xylidin and sufficient alkali to 10 give the ore pulp a distinct alkaline reaction, and subjecting the resulting mixture

to a flotation operation; substantially as described.

4. The method of effecting the concentration of minerals by flotation, which comprises adding to the mineral pulp a small amount of xylidin and of oil, and subjecting the resulting mixture to a flotation operation; substantially as described.

In testimony whereof I affix my signature. 20

CLEMENT L. PERKINS.